

## UNITED STATES PATENT OFFICE.

ISAAC M. SCOTT AND SAMUEL PEACOCK, OF WHEELING, WEST VIRGINIA, AND WILLIAM EARL ARMSTRONG, OF MARTINS FERRY, OHIO, ASSIGNEES TO WHEELING STEEL & IRON COMPANY, OF WHEELING, WEST VIRGINIA, A CORPORATION OF WEST VIRGINIA.

## ELECTROPLATING BATH.

No Drawing.

Application filed February 19, 1923. Serial No. 620,010.

To all whom it may concern:

Be it known that we, ISAAC M. SCOTT, SAMUEL PEACOCK, and WILLIAM EARL ARMSTRONG, all citizens of the United States, the 5 said ISAAC M. SCOTT and SAMUEL PEACOCK residing at Wheeling, in the county of Ohio and State of West Virginia, and the said WILLIAM EARL ARMSTRONG residing at Martins Ferry, in the county of Belmont and 10 State of Ohio, have invented certain new and useful Improvements in Electroplating Baths; and we do hereby declare the following to be a full, clear, and exact description of the invention, such as will enable others 15 skilled in the art to which it appertains to make and use the same.

This invention relates to improvements in electro-tinning and more particularly to the solution of electrolyte, whereby said electro-tinning can be carried out on a commercial scale and in a manner more economical than has been heretofore attained.

With these and other objects in view the invention consists in the novel composition 20 of matter constituting the electrolyte, all as will be more fully hereinafter disclosed and particularly pointed out in the claims.

In order that the precise invention may be 25 more clearly understood it is said:—In the electro-deposition of tin, great difficulty has been heretofore experienced in producing a dense and coherent deposit. This is especially emphasized when the objects to be electro-tinned are constructed of metals 30 higher in the electro-chemical series than is tin, such for example, as steel or iron. Heretofore, articles constructed of metals such as iron, were first electroplated with a metal lower in the electro-chemical series such for 35 example as copper, and upon this last named metal the tin was deposited. But, solutions that are available for depositing the tin directly on iron or steel deteriorate rapidly, and cannot be operated on a commercial 40 scale, economically, unless associated with a suitable restoring solution. These difficulties are all well known in this art.

On the other hand, this invention involves 45 a solution and a method by which electro-tinning can be carried out without difficulty and much more efficiently than heretofore; and this solution can be used for plating

directly on steel and other metals higher in the electro-chemical series. Further, this method may be used for large scale operations with different concentrations and without causing a formation of colloidal or spongy deposits as in the prior procedures. The solutions contain a lower percentage of tin than those heretofore employed, they do 55 not deteriorate or hydrolyze to an objectionable extent, and they operate with almost 100% efficiency. This bath does not require a periodical addition of tin salts as heretofore, or in other words, it is self sustaining. 60

It will be understood by those skilled in the art that the thickness of deposit or amount of tin plated per unit of surface will depend upon the length of time and the 65 number of amperes used, irrespective of the voltage, but of course, the lower the voltage employed the more economical will be the deposition.

It has been found in practice that with 70 say  $\frac{3}{4}$  to  $1\frac{1}{4}$  volts good deposits are obtained with this solution. In carrying out the invention in its preferred form, one may take, for example, 3 parts by weight of a 75 50% commercial hydrofluoric acid (HF) and dissolve therein 1.6 parts by weight of 80 boric acid  $H_3BO_3$ . These acids react with an evolution of heat and form an acid known as fluoboric acid or borofluohydric acid, the simplest formula of which is  $HBF_4$ . In this acid, one dissolves stannous oxide  $SnO$  85 until the acid has taken up the equivalent of 1.35 parts by weight of metallic tin, leaving about 31% of the acid present in the free state.

By this means, there is produced a solution of stannous fluoborate  $Sn(BF_4)_2$ , containing an excess of free fluoboric acid  $HBF_4$ . To increase the conductivity of this solution one adds a metallic salt of a metal higher in the electro-chemical series than iron, and prefers for this purpose the addition of 1.3 parts by weight of aluminum sulphate  $Al_2(SO_4)_3$  or 1.3 parts by weight of magnesium sulphate  $MgSO_4$ . This solution is then diluted with water to such a concentration that it will contain about  $1\frac{1}{3}$  ounces of metallic tin to one gallon. In this diluted solution there is suspended metallic tin as an anode on a positive bus bar and one

2  
suspends the articles to be plated such as sheet steel in the solution and connects them to the negative bus bar whereby on the passage of a suitable electric current, the steel 5 articles become plated with metallic tin.

It has been found it is also desirable to add so-called addition agents or brightening agents, such as molasses, gelatine, etc., to the solution for the purpose of obtaining 10 somewhat improved and bright deposits. It is preferred to use ordinary glue for this purpose and in a quantity of about .03 ounce per gallon of solution, but a larger amount will not interfere with the success of the 15 process. Instead of using stannous oxide  $\text{SnO}$  for introducing the tin into this solution, one may add other tin salts, such as stannous hydrate  $\text{Sn}(\text{OH})_2$  or may dissolve in the solution metallic tin with or without 20 the aid of the electric current. It has been found that the economical addition of tin may also be obtained by suspending metallic tin as anodes in the solution, connected with a positive bus bar and suspending metal 25 strips, surrounded by porous cups in the solution, the metal strips being connected to a negative bus bar. By the passage of a suitable electric current, such as that above disclosed, the tin is dissolved from the 30 anodes into the solution and being unable to pass into the porous cups, it is taken up by the acid. When sufficient tin has been dissolved the cups are removed and the plating 35 continued.

35 We are unable to satisfactorily explain the exact scientific reasons why this solution produces such surprising efficiencies in the coating of tin onto iron, but a plausible explanation resides in the following facts:—  
40 It is well known that the usual bath for electro-depositing tin contains the tin in the form of a sodium stannite or a sodium stannate. It is doubtful if a sodium stannate is in any way useful for tin deposition on 45 iron. It is also well recognized that potash salts are equally inefficient with sodium salts in the electrodeposition of tin on iron. But while these alkali metal tin baths give 50 good initial deposits, they very rapidly hydrolyze in practical use so that after a very small percentage of tin has been deposited a satisfactory coating is no longer obtained. The tin content of these prior baths hydrolyzes in various forms but it is generally 55 accepted that said content separates out in the form of an insoluble meta stannic acid. There is, however, some question as to what is the real form this said insoluble tin actually takes, but there is no dispute as to the 60 fact that it separates out of the solution in a form that makes it no longer available for electro-deposition purposes.

Another fact which makes the alkali tin baths unsatisfactory is that the anode efficiency is very low.

That is, the tin is removed from the solution at an efficiency which is nowhere near a theoretical efficiency if we consider the quantity dissolved from the anodes. It results that for any considerable quantity of 70 tin deposited by the old procedures, fresh additions of alkali tin salts must constantly be added. It is therefore evident that it is only a question of time when the concentration of caustic alkali in the solution will 75 be so great as to preclude any further deposition of tin and this fact alone constitutes a serious objection to the prior procedures.

It is a further recognized fact that with 80 tin depositing salts, in which the tin exists as a base, such for example, as the chlorides or the sulphates, there is also experienced a hydrolytic separation of the tin in forms that are insoluble, and therefore 85 not ionized. It thus again follows that these salts are not utilizable for a satisfactory 90 electrodeposition of metallic tin. Unless these salts are maintained in a very acid solution, this hydrolytic decomposition is so rapid as to preclude the use of such baths 95 for deposition purposes. But on the other hand, if the solution is maintained rather strongly acid, it is impossible to deposit 100 satisfactory coherent tin coatings on metallic iron or steel, because of the action of the acid upon the iron or steel articles. That is, although the deposit may be made, it is very spongy and does not adhere.

There have also been tin baths proposed 100 in which cyanides are employed, and while these baths serve somewhat better than the alkali tin salts for depositing on iron, yet, 105 they are dangerous in practical operations, because stannic acid is capable of setting free prussic acid which is very poisonous and highly dangerous to the operatives. But even if this danger were obviated for 110 which no means are known at this time, the bath is still unsatisfactory in practice due to an excessive hydrolytic decomposition of 115 the tin.

It has further been proposed to use baths 120 of tin containing alkali fluorides. While these baths have a somewhat higher anode efficiency than the baths in which tin is present as a base, yet, they still fail to deposit in large scale operations on iron or steel a satisfactory firmly adherent reguline deposit and are also subject to a very objectionable hydrolytic dissociation.

The bath composed of stannous oxide dissolved in fluoboric acid on the other hand 125 is found to be largely free from the above objections, due probably to the presence of both the boric and the fluoric ions, and so far as is known seems to be the only bath which is not accompanied by an objectionable hydrolytic dissociation. This feature enables this bath to deposit tin on iron and steel in a firmly adherent, reguline coat- 130

ing, which practice proves to be very satisfactory indeed.

In the foregoing description there is disclosed a tin solution in a somewhat diluted form with an acid reaction, but the solution can be used in more concentrated forms such for example as in those having a plurality of times the concentration of that above mentioned. The solution can also be used in the neutral state and for certain purposes one prefers a neutral solution, and such last named solution is especially desirable when chemically pure tin is being deposited.

The above solution has proved satisfactory for the deposition of tin on various metals such as iron, steel and copper, and therefore, it is not desired to be limited to the procedure set forth in the description. This solution and process may also be used with various modifications for numerous purposes that will readily suggest themselves to those skilled in the art without departing from the spirit of our invention.

For example, a conducting metal salt, carbon or other electric conductor may be deposited by well known means in the pores of a fabric or other material and tin may be deposited thereon by following the foregoing procedure. Therefore, it is not desired to be limited to the above disclosure except as may be required by the claims.

What is claimed is:—

1. The herein described electro-plating bath for depositing tin on electric conductors the same consisting essentially of a solution of stannous fluoborate. 35

2. The herein described electro-plating bath for depositing tin on electric conductors the same consisting essentially of a solution of stannous fluoborate admixed with the salt of a metal electro-positive to iron. 40

3. The herein described electro-plating bath for depositing tin on iron or steel the same consisting of a solution of stannous fluoborate admixed with a salt of a metal electro-positive to iron and containing free boro-fluohydric acid. 45

4. The herein described electro-plating bath for depositing tin on iron or steel the same consisting of a solution of stannous fluoborate admixed with aluminum sulphate. 50

5. The herein described electro-plating bath for depositing tin on iron or steel the same consisting of a solution of stannous fluoborate admixed with aluminum sulphate and a substantial percentage of free boro-fluohydric acid. 55

In testimony whereof we affix our signatures.

ISAAC M. SCOTT.

SAMUEL PEACOCK.

WILLIAM EARL ARMSTRONG.